

(Specimens.)

C. M. HALL.

PROCESS OF REDUCING ALUMINUM BY ELECTROLYSIS.

No. 400,766.

Patented Apr. 2, 1889.



Fig 2.



Witnesses:

George E. Hall.  
R. S. Fenwick.

Inventor:  
Charles M. Hall  
Lyons Atty  
Mason, French & Lawrence

# UNITED STATES PATENT OFFICE.

CHARLES M. HALL, OF OBERLIN, OHIO.

## PROCESS OF REDUCING ALUMINIUM BY ELECTROLYSIS.

SPECIFICATION forming part of Letters Patent No. 400,766, dated April 2, 1889.

Application filed July 9, 1886. Serial No. 207,601. (Specimens.)

*To all whom it may concern:*

Be it known that I, CHARLES M. HALL, a citizen of the United States, residing at Oberlin, in the county of Lorain and State of Ohio, have invented certain new and useful Improvements in the Process of Reducing Aluminium by Electrolysis; and I do hereby declare the following to be a full, clear, and exact description of the invention, such as will enable others skilled in the art to which it appertains to make and use the same.

The invention described herein relates to the reduction of aluminium from its oxide by dissolving such oxide in a bath containing a fused fluoride salt of aluminium and then reducing the aluminium by passing an electric current through the bath; and in general terms the invention consists in the electrolysis of a solution of alumina in a fused fluoride salt of aluminium, substantially as herein-after more fully described and claimed.

In the accompanying drawings, forming a part of this specification, Figure 1 is a sectional elevation of a form of apparatus applicable in the practice of my invention; and Fig. 2 is a view, partly in elevation and partly in section, of a modified form of apparatus.

In the practice of my invention I prepare a bath for the solution of the alumina by fusing together in a suitable crucible, A, the fluoride of aluminium and the fluoride of a metal more electro-positive than aluminium—as, for example, the fluoride of sodium potassium, &c.—these salts being preferably mingled together in the proportions of eighty-four parts of sodium fluoride and one hundred and sixty-nine parts of aluminium fluoride, represented by the formula  $Na_2Al_2F_8$ . A convenient method of forming the bath consists in adding to the mineral cryolite of its weight of aluminium fluoride. The object of thus adding aluminium fluoride is to secure in the bath the proper relative proportions of the fluorides of aluminium and sodium. To this fused bath is added alumina or the oxide of aluminium in sufficient quantities, and the alumina being dissolved by the fused bath an electric current is passed through the solution, by means of suitable electrodes, C and D, connected with a dynamo-electric machine or other suitable source of electricity and immersed in the solution. By the action of the

electric current, which preferably has an electro-motive force of about four to six volts, oxygen is released at the positive electrode C, and aluminium is reduced at the negative electrode D, which, on account of the affinity of aluminium for other metals, is formed of carbon when it is desired to produce pure aluminium. The positive electrode may be formed of carbon, copper, platinum, or other suitable material. When formed of carbon, the electrode C is gradually consumed, and must therefore be renewed from time to time; but when formed of copper an oxide coating is formed over the surface of the electrode. This coating serves to protect the electrode from further destruction by the action of the oxygen, but does not interfere materially with the conducting qualities of the electrode.

On account of the affinity of aluminium for other metals, and also the corrosive action of the materials forming the bath on earthy materials, I prefer to form the crucible or melting-pot A of metal—as iron or steel—and protect the same from the action of the aluminium by a carbon lining, A'. This crucible is placed in a suitable furnace, B, and subjected to a sufficient heat to fuse the materials placed therein, such materials fusing at approximately the same temperature as common salt.

In lieu of the electrode D, as shown in Fig. 1, the carbon lining A' may be employed as the negative electrode, as shown in Fig. 2, the conductor from the negative pole of the electric generator being suitably connected, as shown at N', to such lining.

In order to render the bath or solvent more fusible fluoride of lithium may be substituted for a portion of the fluoride of sodium—as, for example, for one-fourth of the fluoride of sodium an equivalent amount of lithium fluoride by molecular weights may be substituted. Thus twenty-six parts of lithium fluoride displacing forty-two parts of sodium fluoride, the resulting combination contains twenty-six parts of lithium fluoride for every one hundred and twenty-six parts of sodium fluoride and three hundred and thirty-eight parts of aluminium fluoride.

While I consider the proportions of fluorides of sodium and aluminium, and of the fluorides of sodium, lithium, and aluminium,

hereinbefore stated, as best adapted for the purpose, such proportions may be varied within certain limits without materially affecting the operation or function of the bath, as, 5 in fact, any proportions which may be found suitable may be employed. The aluminium as it is reduced at the negative electrode is melted and collects thereon in globules, and then drops down to the bottom of the bath, 10 which is of less specific gravity than the molten aluminium, and can be removed by suitable means; or the bath may be poured out and after being cooled the aluminium may be picked out. 15 As hereinbefore stated, the oxygen is released at the positive electrode, and when the latter is formed of carbon combines therewith, forming carbonic oxide, (CO<sub>2</sub>) the carbon being gradually consumed, and with some 20 salts, more particularly the salts of sodium, carbonaceous material is preferably used in the positive electrode or anode; but when the positive electrode is formed of copper, as is preferable when salts of potassium are employed, 25 a copper-oxide coating is first formed on the electrode, thereby forming a protective covering, free oxygen being subsequently given off at the positive electrode.

No claim is made herein specifically to the 30 use of the fluoride of potassium and aluminium as a bath for the reduction of aluminium, as the same forms the subject-matter of an application filed February 2, 1887, and numbered Serially 226,206; nor does the apparatus 35 described herein with more or less particu-

larity form any part of the invention herein, as the same forms the subject-matter of an application, No. 282,952, filed August 17, 1888.

I claim herein as my invention—

1. As an improvement in the art of manufacturing aluminium, the herein-described process, which consists in dissolving alumina in a fused bath composed of the fluorides of aluminium and a metal more electro-positive than aluminium, and then passing 45 an electric current through the fused mass, substantially as set forth. 40

2. As an improvement in the art of manufacturing aluminium, the herein-described process, which consists in dissolving alumina in a fused bath composed of the fluorides of aluminium and sodium, and then passing an electric current, by means of a carbonaceous anode, through the fused mass, substantially 50 as set forth. 55

3. As an improvement in the art of manufacturing aluminium, the herein-described process, which consists in dissolving alumina in a fused bath composed of the fluorides of aluminium, sodium, and lithium, and then 60 passing an electric current, by means of a carbonaceous anode, through the fused mass, substantially as set forth. 60

In testimony whereof I affix my signature in presence of two witnesses.

CHARLES M. HALL.

Witnesses:

GEORGE E. HALL,  
ROBT. L. FENWICK.